# EUROPEAN PATENT SPECIFICATION

(11) **EP 1 707 284 B1**
(45) Date of publication and mention of the grant of the patent: **02.12.2009**
(21) Application number: 05701668.5
(22) Date of filing: 13.01.2005
(51) Int. Cl.: B21C 37/04, B21C 51/00, B23B 5/12

(54) **METHOD FOR THE PRODUCTION OF DEFECT-FREE CALIBRATED STEEL BARS**
VERFAHREN ZUR HERSTELLUNG VON FEHLERFREIEN KALIBRIERTEN STAHLSTANGEN
PROCEDE DE PRODUCTION DE BARRES EN ACIER CALIBREES ET SANS DEFAUTS

(30) Priority: 23.01.2004 ES 200400139
(43) Date of publication of application: 04.10.2006
(73) Proprietor: CALIBRADOS DE PRECISION, S.A., 08120 La Llagosta (Barcelona) (ES)
(72) Inventor: PASCUAL VENTOSA, Lluis, E-Barcelona (ES)
(74) Representative: Durán Moya, Luis-Alfonso
(86) International application number: PCT/ES2005/000013
(87) International publication number: WO 2005/070578

(56) References cited:
- ES-A1- 397 460
- JP-A- 4 238 621
- JP-A- 57 171 515
- JP-A- 59 142 054
- US-A- 4 037 446
- US-A- 4 545 227
- US-A- 5 582 051

## Description

This invention is intended to provide information about a process for the manufacture of defect-free gauged steel bars and the industrial installation which brings about the aforesaid process.

At the present time processes for the manufacture of gauged steel bars which produce gauged bars intended for the manufacture of mechanical parts complying with specific dimensional diameter and external tolerance characteristics and subjected to crack detection during manufacture in order to avoid bars with defects insofar as is possible, are currently known.

The increase in the requirements applying to gauged bars, which makes it necessary for defects, especially surface defects, particularly surface cracks, to be eliminated, has given rise to a need in this industry for processes and installations for the manufacture of defect-free bars which at the same time have satisfactory characteristics for industrialisation of the process.

At the present time, in the main two processes are known for transforming hot rolled steel, which is the raw material used for manufacture of gauged steel bars, namely cold drawing and turning or peeling of the bars.

In the first case the hot rolled steel, that is the so-called rod, from which the scale produced in hot rolling has been cleaned off, is passed through a die which has a reducing cone and a cylindrical gauging part, leaving the wire rounder and with a particular diameter tolerance of the order of 0.1 mm and a smoother surface.

Installations known as combined drawing machines are used to carry out the method currently known as cold drawing, and these normally comprise the following parts:
- A reel,
- A preliminary straightener,
- A machine for cleaning off scale, using shot blasting or brushes,
- A drawing unit incorporating carriages, in which the die is located and which brings about the reduction in cross-section,
- Two groups of horizontal and vertical straightening rollers between which the crack detection equipment is normally located,
- A synchronised cutting system,
- A roller or nozzle straightening system, which includes a feed, unloading and sorting system.

The crack detection systems using induced currents used in these combined machines are capable of detecting defects having minimum depths of approximately 0.15 mm, with the result that bars shaped by this process may have defects of that depth.

The process of turning bars consists of passing the rod through the heads of multiple static or rotary cutters which by removing turnings reduce the diameter of the rod, leaving it rounder and with lower tolerance, and removing most of the surface defects typical of hot rolled rod with the turnings.

Installations which normally comprise the following components are provided to carry out methods of manufacture using turning:
- Spool
- Preliminary straightener
- Preliminary roller (optional) or rotary straightener
- Cutting system
- Straightening system (optional)

In bar turning units, given the roughness of the rod and/or out-of-roundness, once the rolling operation has been performed no detection equipment is provided prior to turning, as this can be used at the end of the process, with a maximum detection depth of approximately 0.15 mm, if a cleaned straightening system is included.

US Patent 4 545 227 describes an apparatus for dry continuous wire drawing in which the surface flaws of the wire are eliminated after each detection or alternatively they are marked in case of not being possible to be removed. However no feed-back is used in order to eventually change the diameter of the incoming wire.

US Patent 4 037 446 discloses a method of producing bright steel from rolled steel wire providing a first stage of reduction of the diameter of the steel wire by calibration, straightening the wire and imparting to the wire a radial bending force moving in a circle above the wire.

Patents abstracts of Japan 57 171 515 discloses a surface flaw removing method combining an automatic crack finder with an automatic cutting device which cuts the wire surface only in the flaw position before the final winding of the wire.

Patent abstracts of Japan 59 142 054 discloses a method and device for removing surface flaws on wire rods combining a crack detector with a grinding device to remove the surface flaws of the wire.

US Patent 5 582 051 discloses an automatic flaw cutting method, and apparatus for wire-shaped metal, to prevent overlooking of flaws rectifying the twist of a wire-shaped metal drawn from a canon-shaped wire supply stand, applying an automatic flaw-cutting process and removing the uncut flaws by hand.

Patent abstracts of Japan 04 238 621 discloses a device and method for manufacturing wire rod in which the rod is straightened and descaled prior to drawing and flaw detection, removing the flaws by an automatic flaw-repairing device before the spheroidizing and annealing of the wire rod in a treating furnace.

In order to bring about the manufacture of defect-free gauged bars in a suitably industrialised way this invention provides a process in which the hot rolled rod proceeds from the spool to a pre-straightening and subsequent descaling operation, then proceeds to a combined stage of gauging by drawing and an intermediate crack monitoring process to detect the depth of defects in the bar in relation to a calibrated depth, these defects being subsequently removed in a machining operation with turnings being removed to a depth greater than that gauged by the detection equipment. In order to do this the detection equipment is set to a depth corresponding to the defects experimentally detected in the bars and the bars are machined, removing part of the material corresponding to the detection depth plus a specific excess so as to achieve greater safety when wholly cleaning the bar, the said detection zone detecting any areas in which the defects are greater than the gauge for the detection equipment, producing bars which will be automatically separated at the end of the process in accordance with universally known methods for identifying defects in bars of a continuous type in order ultimately to locate bars incorporating defects and to allow them to be eliminated. However, all defects within the gauge value of the detection equipment will be removed automatically in the stage of turning the bars, which will remove a quantity of material corresponding to the gauged depth plus a small safety margin.

The process will therefore make it possible to guarantee that there are no surface defects which can be detected by existing monitoring equipment.

The process to which this invention relates will include the possibility of feeding results back to the cold gauging stage of the installation because if the number of bars rejected during the final stage as a result of intermediate sorting is very high the machining depth will be increased, simultaneously changing the gauging die to a larger diameter to enable the material to have sufficient excess for cracks to be removed, and so that the nominal diameter for the gauged bar can be achieved. Obviously, if no rejects at all are produced, this will mean that the equipment must be gauged to a lower value, avoiding excessive losses of material due to removal of the turnings.

Thus through applying this process and the corresponding installation the absence of surface defects is achieved and losses due to turnings or material rejected because of the depth of defects detected is reduced to a minimum.

For a better understanding some drawings representing this invention are appended by way of a non-restrictive explanatory example.

Figure 1 shows a diagram of the set of components involved in this invention.

Figure 2 shows diagrammatically the interrelationship between bar diameters from the starting rod to the final gauged bar with the corresponding excesses.

As will be seen in Figure 1, the process begins with the spool -1- of hot rolled rod from which the rod is drawn, after which there is a pre-straightening stage 2- and subsequently the stage -3- of eliminating surface residues or scale using shot blasting or brush systems, yielding the straightened and descaled bar - 4- which then goes to a drawing gauging stage which incorporates a die and a pulling unit represented by the number -5-. The gauged rod -6- then goes onto the control system -7- which is calibrated to detect cracks at a particular depth, identifying those locations on the continuous bar where areas having defects greater than the machine's gauge have been located. The gauged rod then passes to the machining system -8- in which a surface part of the bar which is slightly greater than the gauge for the monitoring system is removed mechanically, with the result that surface defects are systematically removed. The rod then passes to the cutting stage -9-, after which it is passed to the straightening unit -10-, passing finally through the bar selection zone -11- where bars which fulfil the specified conditions -12- are regarded as being marketable bars and defective bars -12'- in which defects of depth greater than the machine gauge have been detected will be eliminated.

Figure 2 shows diagrammatically the process in which will be seen the diameter -φb- of the rod after cold drawing incorporating multiple defects due to surface cracks such as -d1-, -d2-, -d3-, etc., which lie within the gauge value □A□ for the machine. It is possible that some defects such as -d4- will be greater than the gauge value, giving rise to a reference mark in the detection zone which will bring about automatic rejection of the bar at the end of the line. The crack detection machine is calibrated to the value -A- indicated in the graph, and turning is carried out with removal of the excess -B- which comprises the gauge -A- plus a small safety surplus -ε- shown in the graph, giving rise finally to the nominal diameter -φₙ- of the bar which it is desired to obtain.

If the number of bars rejected because of cracks is excessive, information can be fed back, with the bars being rolled to a diameter -φ_{b}- which is slightly larger so that the excess turned off -B- can be increased, eliminating the defects and producing defect-free bars at the end of the process. If this is not the case, that is, if the gross diameter -φ_{b}- can be reduced, the opposite is carried out during the rolling stage, the excess of material with respect to the nominal diameter -φB- being decreased.

Finally, through applying the process in the installation to which the invention relates the complete absence of surface defects is achieved in a wholly industrialised way, bringing about minimum loss from turnings or materials rejected in the unit.

## Claims

1. Process for the manufacture of rolled steel bars of the type comprising feeding a rolling line from a spool of hot rolled rod **(1)** with a pre-straightening **(2)** and descaling stage **(3),** followed by gauging through drawing **(5),** crack monitoring **(7)** and cutting **(9)** and straightening **(10),** with a final sorting **(11)** into acceptable **(12)** and unacceptable bars **(12'), characterised in that** the operation of gauging by drawing **(5)** is combined with a subsequent stage of monitoring and identifying cracks **(7)** and a subsequent operation **(8)** of mechanically machining the bar **(4)** through the removal of turnings prior to cutting **(9)** of the bars in such a way that the gauged depth for the detection of cracks has a value corresponding to the surface defects in the bar and somewhat less than the machining depth in the subsequent stage **(8)** of machining the bar, giving rise to feedback of information on the percentages of bars rejected **(12')** because of cracks in the final sorting of the bars to the stage of gauging by drawing **(5)** and the machining stage **(8)** in order to readjust the rolling and machining diameters.

2. Process for the manufacture of rolled steel bars according to claim 1, **characterised in that** if the percentage of bars **(12')** eliminated because of cracks in the final sort **(11)** is higher than a specified control value the external diameter when roughing out the rod **(1)** and the machining depth **(8)** is increased in order to allow elimination of the defective bars.

3. Process for the manufacture of rolled steel bars according to claim 1, **characterised in that** the diameter of the rough rod **(1)** and the machining depth during the stage **(8)** of machining the bar are reduced if the reduction in defects in the bars in the final sort **(11)** makes it possible to reduce the excess material removed by peeling.

## Patentansprüche

1. Verfahren zum Herstellen von gewalzten Stahlstäben, umfassend: von einer Spule mit warm gewalztem Stangenmaterial (1) wird eine Walzstraße mit einer Vorrichtstufe (2) und einer Entzunderungsstufe (3) beschickt, gefolgt von einem Eichen durch Ziehen (5), einer Rissüberwachung (7) und Schneiden (9) sowie Richten (10) mit abschließender Sortierung (11) in akzeptierbare (12) und nichtakzeptierbare (12') Stäbe, **dadurch gekennzeichnet, dass** der Vorgang des Eichens durch Ziehen (5) kombiniert ist mit einer anschließenden Stufe des Überwachens und Nachweisens von Rissen (7) sowie einem anschließenden Vorgang (8) des mechanischen Zerspanens des Stabs (4) durch Abdrehen vor dem Schneiden (9) der Stäbe derart, dass die Eichtiefe für den Nachweis von Rissen einen Wert aufweist, der den Oberflächendefekten in dem Stab entspricht und etwas kleiner ist als die Zerspantiefe der anschließenden Stufe (8) der Zerspanung des Stabs, mit der Folge, dass Informationen über die prozentualen Anteile der Stäbe, die aufgrund von Rissen bei der abschließenden Sortierung der Stäbe zurückgewiesen (12') wurden, zu der Stufe des Eichens durch Ziehen (5) und zu der Zerspanungsstufe (8) zurückgeführt werden, um die Walz- und Zerspandurchmesser neu einzustellen.

2. Verfahren zum Herstellen von gewalzten Stahlstäben nach Anspruch 1, **dadurch gekennzeichnet, dass** dann, wenn der Prozentsatz von Stäben (12'), die aufgrund von Rissen bei der abschließenden Sortierung (11) eliminiert werden, höher ist als ein spezifizierter Kontrollwert, der Außendurchmesser beim Aufrauhen des Stangenmaterials (1) und die Zerspantiefe (8) erhöht werden, um eine Eliminierung defekter Stäbe zu ermöglichen.

3. Verfahren zum Herstellen von gewalzten Stahlstäben nach Anspruch 1, **dadurch gekennzeichnet, dass** der Durchmesser des rauhen Stangenmaterials (1) und die Zerspantiefe während der Zerspanstufe (8) des Stabs verringert werden, wenn die Reduzierung von Defekten in den Stäben bei der abschließenden Sortierung (11) die Möglichkeit bietet, das durch Abschälen beseitigte überschüssige Material zu verringern.

## Revendications

1. Procédé pour la fabrication de barres d'acier laminés du type comprenant l'alimentation d'une ligne de laminage à partir d'une bobine de tige laminée à chaud (1) avec une étape de pré-dressage (2) et de décalaminage (3), suivie du calibrage par étirage (5), du contrôle des fissures (7) et de la coupe (9) et du dressage (10), avec un tri final (11) en barres acceptables (12) et en barres inacceptables (12'),
**caractérisé en ce que** l'opération de calibrage par étirage (5) est combinée à une étape ultérieure de contrôle et d'identification de fissures (7) et d'une opération ultérieure (8) d'usinage mécanique de la barre (4) par l'enlèvement des copeaux de tournage avant la coupe (9) des barres, de telle sorte que la profondeur calibrée pour la détection des fissures a une valeur correspondant aux défauts de surface dans la barre et quelque peu inférieure à la profondeur d'usinage dans l'étape ultérieure (8) d'usinage de la barre, donnant lieu au retour d'information sur les pourcentages de barres rejetées (12') en raison de fissures dans le tri final des barres à l'étape de calibrage par étirage (5) et l'étape d'usinage (8), afin de réajuster les diamètres de laminage et d'usinage.

2. Procédé pour la fabrication de barres d'acier laminés selon la revendication 1, **caractérisé en ce que**, si le pourcentage des barres éliminées (12') en raison de fissures dans le tri final (11) est supérieur à une valeur de contrôle spécifiée, on augmente le diamètre extérieur lors du dégrossissage de la tige (1) et la profondeur d'usinage (8) pour permettre l'élimination de lingots défectueux.

3. Procédé pour la fabrication de lingots d'acier laminé selon la revendication 1, **caractérisé en ce que** le diamètre de la tige brute (1) et la profondeur d'usinage pendant l'étape (8) d'usinage de la barre sont réduits si la réduction de défauts dans les barres dans le tri final (11) permet de réduire le matériau excédentaire enlevé par écroûtage.
